

# UNITED STATES PATENT OFFICE.

JOHN F. A. MUMM, OF DAYTON, KENTUCKY.

## EXPLOSIVE COMPOUND.

SPECIFICATION forming part of Letters Patent No. 417,577, dated December 17, 1889.

Application filed September 24, 1889. Serial No. 324,923. (No specimens.)

*To all whom it may concern:*

Be it known that I, JOHN F. A. MUMM, of Dayton, in the county of Campbell and State of Kentucky, have invented a new and useful Improvement in Explosive Compounds, of which the following is a full, clear, and exact description.

This invention consists in a new composition of matter or explosive compound suitable for railway fog-signals or torpedoes, for charging bombs and grenades, and for blasting and shooting purposes.

My composition consists of the following ingredients, combined in or about the proportions stated, viz: chlorate of potash, one pound, (sixteen ounces;) antimony, (pure needle-powdered,) eight ounces; charcoal, one ounce; refined flowers of sulphur, two ounces; glycerine, one ounce; collodion, one ounce; sulphuric acid, four drops; nitric acid, two drops; alcohol, three ounces; water, two to three ounces.

In the preparation of this compound I first put the alcohol and water in a mortar and then add thereto the glycerine and the sulphuric and nitric acids and mix the whole together. I then introduce into this mixture the chlorate of potash and allow it to soak for a short time. In a separate vessel or mortar I also mix the antimony, charcoal, and flowers of sulphur, and thoroughly grind or pound them dry, and add such materials to the soaked chlorate of potash and slightly mix the whole. I next introduce the collodion to the several ingredients of this combined mixture and thoroughly mix or grind the whole together. Should the collodion be introduced in advance of the other ingredients, it would become cottony; but adding it at the last this is avoided. The compound thus prepared I usually put with a tablespoon, in quantities of about two ounces weight, onto boards covered with pasteboard or other paper, to remove moisture by absorption, which operation may be repeated upon another like-covered board till the compound is dry and ready to put up for use. For railway fog-signals or torpedoes I usually put it up in tin boxes lined with waxed manila tissue-paper to keep the box from rusting and the composition dry, and to give increased

safety during transportation, by keeping the metal surface of the box free from contact and friction with it. Said box, however, is not wholly filled with the compound, but the latter has placed upon the top of it a frictional substance, as usual in torpedo-like signals, to provide for the fulminate being more readily ignited—such as a few loose pieces of broken glass, in preference to pellets—after which the whole is covered with waxed manila paper and the box closed as tight as it is practicable to make it.

To use the compound for making bombs or grenades, it should be put in the shells with a leather or rubber funnel and provision made for lighting the explosive either by a fulminate cap or by a time-fuse.

For blasting purposes, the compound should be put up in cartridge-shells and the same be exploded either by electricity or fuse.

For gunning or shooting purposes, the compound should not be used loose, but in cartridges, which may be exploded by fulminate caps. It may be used for guns of all kinds, including fowling-pieces, rifles, revolvers, and cannons.

The compound will be found to be much more powerful than ordinary gunpowder, safer to make and handle than dynamite, nitro-glycerine, and the like, and is not liable to separate.

I am aware that several of the ingredients named in this compound have before been used in different combinations for the making of explosives. Such, therefore, separately considered, I do not claim.

Having thus described my invention, what I claim as new, and desire to secure by Letters Patent, is—

The within-described explosive compound, made of or from a mixture of the following ingredients, substantially in the proportions specified, to wit: chlorate of potash, antimony, charcoal, flowers of sulphur, glycerine, collodion, sulphuric acid, nitric acid, alcohol, and water.

JOHN F. A. MUMM.

Witnesses:

ARTHUR J. SMITH,  
R. B. WILSON.